

## UNITED STATES PATENT OFFICE.

WILLIAM R. VEAZEY, OF CLEVELAND HEIGHTS, OHIO, ASSIGNOR TO THE DOW CHEMICAL COMPANY, OF MIDLAND, MICHIGAN, A CORPORATION OF MICHIGAN.

## MAGNESIUM ALLOY AND METHOD OF MAKING SAME.

No Drawing.

Application filed December 8, 1924. Serial No. 754,464.

The present improved alloy is one in which magnesium is the predominant element, the object being to develop an alloy that will possess the characteristic lightness which is obtained by the use of magnesium in excess of eighty per cent, while such alloy will be characterized by high strength and toughness as well as possess a sufficient degree of hardness. More particularly such alloy consists of magnesium and from several hundredths to several tenths per cent of vanadium.

It has not been found feasible to heat the metals in question together for the purpose of alloying the same, since this will involve the use of a temperature above the boiling point of magnesium, the melting point of vanadium being approximately 1715 degrees centigrade. By the present improved method, however, it has been found possible to produce alloys of these two metals containing substantial amounts of vanadium corresponding with the amount for instance employed in so-called vanadium steels and exercising a marked influence in the resultant product. Such product having a vanadium content of less than one per cent is for all practical purposes no heavier than pure magnesium, which of course is very much lighter than aluminum and the commercial aluminum alloys; at the same time if properly cast such alloy is of considerably greater tensile strength and impact-toughness without being unduly hard.

The invention then consists of a new product containing magnesium and vanadium in approximately the proportions stated, together with the steps involved in the making of such alloys hereinafter fully described and particularly set forth in the claims. The following description it will be understood thus sets forth but several of various ways in which the invention may be carried out.

Briefly stated, the improved method of making the alloy in hand consists in inter-fusing a limited amount of a suitable vanadium compound with an excess of magnesium whereby such compound is reduced to the metal and thereupon forms an alloy with the residuum of magnesium still largely exceeding the amount of the vanadium thus reduced from the compound employed.

Preferably vanadium pentoxide ( $V_2O_5$ ) is employed, which compound may be prepared most conveniently from ammonium vanadate ( $NH_4VO_3$ ). Such preparation is accomplished by igniting the vanadate and then fusing the resulting red-yellow powder in a suitable crucible, the resulting product being a red liquor which on solidifying becomes a dense dark red crystalline substance, melting at about 680 degrees centigrade. (Thorpe).

A mass of molten magnesium is then prepared preferably using a flux of slightly greater specific gravity than the molten metal and having sufficient surface tension to cause it to form a film thereover and thus prevent exposure of the metal to the atmosphere. The vanadium pentoxide is then added to such molten magnesium being pushed under the surface thereof since it exhibits a tendency to float and if necessary a thorough intermixture of the oxide may be insured by stirring. However, the reaction of the magnesium with the oxide occurs almost immediately, the latter being reduced to metallic form and incorporated in the mass of molten magnesium to form the desired alloy.

The molten alloy may then be conveniently removed from the crucible or melting pot by means of an ordinary ladle and is cast into bars or such other shapes as may be desired. The amount of vanadium derived from any given quantity of the oxide is per cent but some of this apparently is lost in the reaction, at least less than the theoretical amount of vanadium appears in the final alloy. However, the amount of oxide that requires to be added to give an alloy containing the desired number of hundredths per cent of vanadium may be readily calculated, as need not be explained in detail. The amount of such alloying ingredient actually introduced may be checked by analysis using the method ordinarily employed in the analysis of chrome-vanadium steels. From three (3) one-hundredths per cent to fifteen (15) one-hundredths per cent of vanadium have been found to give most satisfactory results.

Other modes of applying the principle of my invention may be employed instead of the one explained, change being made as

regards the composition and method herein disclosed, provided the ingredients or steps stated by any of the following claims or the equivalent of such stated ingredients or steps be employed.

I therefore particularly point out and distinctly claim as my invention:—

1. As a new product, an alloy containing magnesium as the predominant component 10 and vanadium as a relatively small modifying-component.

2. As a new product, an alloy containing magnesium and vanadium, wherein the magnesium is the predominant component and 15 the vanadium is present in substantial amount but less than one per cent.

3. As a new product, an alloy consisting of magnesium and from several hundredths to several tenths per cent of vanadium.

20 4. As a new product, an alloy consisting of magnesium and approximately fifteen (15) hundredths per cent of vanadium.

5. The method of making an alloy of vanadium with magnesium, which consists 25 in interfusing with an excess of magnesium an amount of a vanadium compound adapt-

ed to be reduced to metallic alloy state in the magnesium.

6. The method of making an alloy of vanadium with magnesium, which consists 30 in interfusing with an excess of magnesium an amount of vanadium pentoxide to be reduced to metallic state in the magnesium.

7. The method of making an alloy of vanadium with magnesium, which consists 35 in adding to a body of magnesium in molten state an amount of vanadium compound in excess of that required to reduce such compound, whereby the desired proportion of metallic vanadium is alloyed in such magnesium.

8. The method of making an alloy of vanadium with magnesium, which consists in adding to a body of magnesium in molten state an amount of vanadium pentoxide in 45 excess of that required to reduce such compound, whereby the desired proportion of metallic vanadium is alloyed in such magnesium.

Signed by me, this 4th day of December, 50  
1924.

WILLIAM R. VEAZEY.